# EUROPEAN PATENT SPECIFICATION

(11) **EP 0 456 413 B1**
(45) Date of publication and mention of the grant of the patent: **28.06.1995**
(21) Application number: 91303976.4
(22) Date of filing: 02.05.1991
(51) Int. Cl.: C09C 1/02, B41M 5/30, B41M 5/40

(54) **Calcium carbonate pigment for heat-sensitive recording paper, process for preparing same, coating composition for heat-sensitive recording paper and heat-sensitive recording paper**
Kalziumkarbonatpigment für wärmeempfindliches Aufzeichnungspapier, Verfahren zu dessen Herstellung, Mischung zur Beschichtung von wärmeempfindlichem Aufzeichnungspapier und wärmeempfindliches Aufzeichnungspapier
Carbonate de calcium pigmentaire pour papier d'enregistrement thermosensible, procédé de préparation, composition de revêtement pour papier d'enregistrement thermosensible et papier d'enregistrement thermosensible

(30) Priority: 11.05.1990 JP 122517/90
(43) Date of publication of application: 13.11.1991
(73) Proprietor: SHIRAISHI CENTRAL LABORATORIES, CO. LTD., Amagasaki-shi, Hyogo 600 (JP)
(72) Inventor: Tsukisaka, Ryogo, Takarazuka-shi, Hyogo-ken (JP); Kondo, Satoshi, Amagasaki-shi, Hyogo-ken (JP); Kaneguchi, Toshio, Kobe-shi, Hyogo-ken (JP); Sakamoto, Atsushi, Yao-shi, Osaka-fu (JP)
(74) Representative: Ede, Eric

(56) References cited:
- GB-A- 684 016
- US-A- 2 198 223
- US-A- 5 007 964
- WORLD PATENTS INDEX, Week 47, Derwent Publications Ltd., London, GB; AN 79-84890B/47; & JP-A-54 131 599

## Description

### BACKGROUND OF THE INVENTION

The present invention relates to an anti-fogging and surface-treated calcium carbonate pigment for the coating layer of heat-sensitive recording paper, a process for preparing the same, a coating composition comprising the calcium carbonate for heat-sensitive recording paper, and heat-sensitive recording paper coated with the composition.

Calcium carbonates include light calcium carbonate and heavy calcium carbonate which are up to 10 m²/g in BET specific surface area, and fine calcium carbonate in excess of 10 m²/g in BET specific surface area. Calcium carbonate is widely used as a pigment for papers, coating compositions, inks, etc. and also as a filler for rubbers, plastics, papers, sealing materials, etc.

In recent years, calcium carbonate is increasingly used also as a pigment for the coating layer of information recording papers such as heat-sensitive recording paper, ink-jet recording paper, etc.

Calcium carbonate is incorporated into coating compositions for heat-sensitive recording paper generally in order to improve the whiteness, non-transparency, surface-smoothness, writablity and like properties of heat-sensitive recording paper as in the case of usual papers. Yet the main object of incorporation of the calcium carbonate is to give the following effects. When heat-sensitive recording paper is heated by the thermal head of a heat-sensitive facsimile system or heat-sensitive printer to develop a color for recording, a higher fatty acid amide or like chromogenic sensitivity adjusting agent, crystal violet lactone or like dye, etc. adhere to the thermal head as residual matter (hereinafter referred to as "residue") to obscure the recorded characters or to reduce the runnablity, i.e., the ability of recording paper to smoothly pass, so that calcium carbonate is incorporated in the coating composition for such paper to inhibit or prevent the adhesion of the residue (hereinafter referred to as "effect to remove residue") and also to achieve heat transfer with enhanced efficiency from the thermal head to the surface of heat-sensitive recording paper.

Heat-sensitive recording paper is a recording material comprising a chromogenic material, a color developer, a pigment and other components, and is required to have:
(1) an ability to give an image of distinct color;
(2) a background having high whiteness, i.e. free of fogging;
(3) an ability to produce an image exhibiting a high weatherability even during long-term storage.

Use of highly oil-absorbent calcium carbonate pigment has been considered desirable for improvement of the effect to remove residue. Such known calcium carbonates include, for example, bodies of intertwined needle- to pillar-like calcium carbonate particles as disclosed in Japanese Examined Patent Publication No.8048/1988 and highly oil- and water-absorbent calcium carbonate as described in Japanese Unexamined Patent Publication No.230424/1989. These calcium carbonates are excellent in the effect to remove residue, but are not always fully satisfactory in anti-fogging property, ability to form images with high resistance to weather, especially to light, heat transfer efficiency, etc.

Currently attempts are being made in the art to develop a heat-sensitive recording paper which is able to achieve speedy recording, and there is a tendency to use more highly oil-absorbent calcium carbonates capable of producing an improved effect to remove residue and giving a higher heat transfer efficiency. Nevertheless calcium carbonate has yet to be developed which is fully satisfactory in anti-fogging property of heat-sensitive recording paper, ability to form images of high weatherability, etc.

It is an object of the invention to provide a calcium carbonate pigment which is sufficiently highly oil-absorbent to provide an improved effect to remove residue, and also outstanding in anti-fogging property, ability to form images of high weatherability, etc.

We thought that the above object might be accomplished by surface-treating a highly oil-absorbent calcium carbonate pigment with a certain substance. For investigation, we conducted extensive research to provide a surface-treated calcium carbonate which, when used as a pigment for the coating layer of heat-sensitive recording paper, exhibits not only an excellent effect to remove residue and a high chromogenic sensitivity, but also an excellent property of forming images of high weatherability with substantially no fogging. As a result of the research, we found the following. When a specific calcium carbonate surface-treating agent is added to an aqueous suspension of calcium carbonate particles having a BET specific surface area of about 17 to about 55 m²/g, and the mixture is stirred to surface-treat the carbonate, the thus treated carbonate is given a surface acidity of solid of about 33 to about 38 »mol/g with substantially no reduction of oil absorption of the starting calcium carbonate, and is rendered able to achieve remarkable effects unattainable by known calcium carbonates. The present invention has been accomplished based on this novel finding.

According to the present invention, there is provided a calcium carbonate pigment for heat-sensitive recording paper, the pigment having a BET specific surface area of 17 to 55 m²/g, preferably 19 to 55 m²/g, an oil absorption of 90 to 220 ml/100 g as determined by the Ogura method and a surface acidity of solid represented by the equation (Z):

$\text{y=0.13 x + 31 (Z)}$

wherein x is a BET specific surface area (m²/g) and y is a surface acidity of solid (»mol/g).

The present invention also provides a process for preparing the foregoing calcium carbonate pigment for heat-sensitive recording paper, the process comprising the steps of (i) adding a calcium carbonate surface-treating agent to an aqueous suspension of calcium carbonate having a BET specific surface area of 17 to 55 m²/g, preferably 19 to 55 m²/g, the surface-treating agent being at least one member selected from the group consisting of hydroxide of alkaline earth metal, hydroxide of alkali metal, carbonate of alkali metal, bicarbonate of alkali metal, sodium aluminate, aluminum acetate and C₄₋₁₄ aliphatic amine acetate; and (ii) stirring the mixture.

The invention further provides a coating composition for heat-sensitive recording paper characterized in that the composition contains the above calcium carbonate pigment for heat-sensitive recording paper.

Throughout the specification and claims, the BET specific surface area was determined by the low-temperature nitrogen adsorption method (see "Particle Size Determination Techniques," edited by the Research Association of Powder Technology, Nikkan Kogyo Press, 1st edition, 1975, pp. 299-305). The surface acidity of solid was determined by an amine titrimetric determination method (see Kozo Tabe and Tsuneichi Takeshita, "Acid-base Catalyst," Sangyo Tosho, 1st edition, 1966, pp.164-167). The method comprises titrating a calcium carbonate pigment as a solid acid in benzene with p-dimethylamino-azobenzene (dimethyl yellow) as an indicator using normal butyl amine. The oil absorption was determined by the Ogura method (see Junzo Matsumoto and Masateru Ogura, "Pigments, Coloring Materials and Inks," Kyoritsu Shuppan Co., Ltd., 4th print, 1950, pp. 66-67, with use of boiled linseed oil according to JIS K 5421).

Table 1 below shows the physical properties of the calcium carbonate pigment of the invention for heat-sensitive recording paper in comparison with those of known calcium carbonates.

The known calcium carbonates (i) to (iv) listed in Table 1 are as follows.
(i) Highly oil- and water-absorbent calcium carbonate as disclosed in Japanese Unexamined Patent Publication No.230424/1989
(ii) Fine precipitated calcium carbonate
(iii) Light calcium carbonate
(iv) Bodies of intertwined needle-like to pillar-like calcium carbonate particles as disclosed in Japanese Examined Patent Publication No.8048/1988

The properties such as bulk in Table 1 were determined by the following methods.
- Bulk:: Pigment-testing method according to JIS K 5101
- Sedimentation volume:: 5 g of calcium carbonate was placed into a 100 ml measuring cylinder, and water was added to make 100 ml of a suspension. After shaking for 20 seconds, the suspension was left to stand for 60 minutes to determine the volume of sediment.
- Hiding power:: Pigment-testing method according to JIS K 5101
- True specific gravity:: Pigment-testing method according to JIS K 5101
- Crystal system:: Determined by X ray diffraction method
- Mean particle size:: Median particle size as measured by light transmission particle size determination method.

Table 1 shows that the surface-treated calcium carbonate pigment of the invention has a surface acidity of solid of as low as 33 to 38 »mol/g compared with the known calcium carbonate (i) having a BET specific surface area of about 25 to 55 m²/g, and retains high oil absorption which is another important property of calcium carbonate pigment for heat-sensitive recording paper.

Our research revealed that calcium carbonate having a BET specific surface area of about 17 to about 55 m²/g has the problem of being generally not always satisfactory in the anti-fogging property presumably because of its high surface acidity of solid due to its great BET specific surface area irrespective of the other physical properties such as particle shape, sedimentation volume, etc. In other words, generally calcium carbonates having a BET specific surface area of about 17 to about 55 m²/g would be likely to cause fogging when used as a pigment for heat-sensitive recording paper. Therefore the surface-treating method of the invention shows a particular significance when employed to treat calcium carbonates having a BET specific surface area of 17 to 55 m²/g, preferably 19 to 55 m²/g. The method of the invention reduces the surface acidity of solid of calcium carbonate to the specific range of 33 to 38 »mol/g in the specific relation represented by the above-defined equation (Z) with substantially no decrease in the BET specific surface area or in the oil absorption.

Now we turn to the properties of the calcium carbonate pigments of the invention. The calcium carbonate pigments less than 17 m²/g in BET specific surface area have an inherently low surface acidity of solid like the starting calcium carbonate and are virtually free of fogging problem, but tend to have a low effect to remove residue because of generally low oil absorption. On the other hand, the treatment of calcium carbonate pigments more than 55 m²/g in BET specific surface area requires an increased amount of a surface-treating agent which is needed in order to diminish the high surface acidity of solid of the starting calcium carbonate to 38 »mol/g as specified above according to the equation (Z), so that the obtained calcium carbonate tends to have a decreased oil absorption. Therefore such calcium carbonates are undesirable. To give a surface acidity of solid of less than 33 »mol/g to calcium carbonate, an increased amount of surface-treating agent is required, resulting in reduction of oil absorption. Thus such calcium carbonates are undesirable. In this case, presumably due to the relatively high surface basicity of solid, the obtained heat-sensitive recording paper is apt to form images of low weatherability. Above 38 »mol/g of a surface acidity of solid, a fogging problem may arise.

The calcium carbonate pigment of the invention is usually prepared by the following process. To an aqueous suspension of calcium carbonate having a BET specific surface area of 17 to 55 m²/g is added at least one calcium carbonate surface-treating agent selected from the group consisting of hydroxide of alkaline earth metal, hydroxide of alkali metal, carbonate of alkali metal, bicarbonate of alkali metal, sodium aluminate, aluminum acetate and acetic acid salt of C₄₋₁₄ aliphatic amine. Then the mixture is stirred to treat the surface of the pigment particles.

Useful starting calcium carbonates having a BET specific surface area of 17 to 55 m²/g include a variety of known calcium carbonates. Among them, it is desirable to use those as disclosed in Japanese Unexamined Patent Publication No.230424/1989 and Japanese Examined Patent Publications No.31530/1982 and No.30815/1982.

More desirable among these starting calcium carbonate pigments are the calcium carbonate pigment as disclosed in Japanese Unexamined Patent Publication No.230424/1989 which is 25 to 55 m²/g in BET specific surface area, between 5 and 110 in the ratio of BET specific surface area (m²/g)/mean particle size (»m), at least 120 ml/100 g in oil absorption as determined by the Ogura method and at least 1.8 g/g in water absorption, and the calcium carbonate pigment which is 17 to 55 m²/g, preferably 19 to 55 m²/g, in BET specific surface area, among the bodies of intertwined needle-like calcium carbonate particles as disclosed in Japanese Examined Patent Publication No.31530/1982, the particles being formed of bodies of needle-like primary particles of calcium carbonate three-dimensionally intertwined irregularly and having mean dimensions of 0.5 to 10 »m in length (L) and 0.05 to 0.2 »m in width (W) as observed under an electron microscope, an aspect ratio (L/W) of from 10 to 50, a void volume of 1.8 to 3.3 ml/g as measured by a porosimeter (mercury intrusion porosimetry) and an oil absorption of 50 to 100 ml/100 g as measured according to JIS K 5101.

The oil absorption of calcium carbonate pigment contributes to the effect to remove residue. From the viewpoint of the effect to remove residue, it is suitable in the invention to use starting calcium carbonate pigments of preferably 90 to 220 ml/100 g, more preferably 93 to 220 ml/ 100 g, in oil absorption. It is preferable that the starting calcium carbonate pigments are those having a bulk of 6.5 to 15 ml/g, preferably 7 to 15 ml/g.

Of calcium carbonate surface-treating agents useful in the invention, typical hydroxides of alkaline earth metals are hydroxides of magnesium, calcium or like metals, preferable hydroxides, carbonates or bicarbonates of alkali metals are sodium or potassium hydroxides, carbonates or bicarbonates, and preferred C₄₋₁₄ aliphatic amine acetic acid salts are butyl amine, octyl amine and lauryl amine acetic acid salts. The amount of the calcium carbonate surface-treating agent which is added to the aqueous suspension of calcium carbonate of 17 to 55 m²/g in BET specific surface area is in the range of 0.1 to 5 parts by weight, preferably 0.2 to 4 parts by weight, per 100 parts by weight of the calcium carbonate. When the amount is less than 0.1 part by weight, the surface acidity of solid can not be suppressed as contemplated and the heat-sensitive paper incorporating the treated carbonate is not imparted an improved anti-fogging property. When the amount is more than 5 parts by weight, the obtained heat-sensitive paper has an improved anti-fogging property but tends to have an impaired effect to remove residue due to reduced oil absorption. Therefore the amount of surface-treating agent outside the above range is undesirable.

The concentration of solids in the aqueous suspension of starting calcium carbonate is not specifically limited, but is usually in the range of 5 to 30% by weight, preferably 7 to 25% by weight. The mixture is stirred for surface treatment preferably at a temperature of 15 to 35°C. The aqueous suspension of starting calcium carbonate is stirred by stirring means which can stir uniformly the whole suspension, such as a propeller-type stirrer, high-speed impeller dispersing means, an oar-type stirrer, turbine-type stirrer, a stirrer of the type capable of blowing air or like gas, etc. The stirring time is not specifically limited, but is preferably in the range of about 10 to about 30 minutes.

The calcium carbonate pigment of the invention having the BET specific surface area and the surface acidity of solid related to each other as represented by the equation (Z) is prepared by surface-treating the starting calcium carbonate of the above-specified BET specific surface area under the above conditions. As compared with the starting calcium carbonate, the obtained calcium carbonate is slightly reduced or increased, but not substantially reduced to an unacceptable degree, in oil absorption, and has suppressed surface acidity of solid in the range of 33 to 38 »mol/g.

The calcium carbonate pigment obtained by the above surface treatment may be used in the form of a paste which is obtained by dewatering the suspension resulting from the surface treatment by a filter press or like dewatering means, or in the form of a powder prepared in the conventional manner by drying the paste, pulverizing the solid and classifying the particles.

The thus obtained calcium carbonate pigment of the invention, when used for forming a coating layer in heat-sensitive recording paper, was found to exhibit, due to the above specific properties of the surface, the excellent properties which have not been found in known calcium carbonates. Therefore, the present invention also relates to coating compositions for heat-sensitive recording paper which comprise about 5 to about 90% by weight of the above-obtained calcium carbonate pigment based on the total solids. Given below are examples of coating compositions of the invention.

### (1) Composition for forming a heat-sensitive recording layer of heat-sensitive recording paper

This composition comprises 5 to 60 wt. % of the calcium carbonate pigment of the invention as admixed with a known colorless to pale-colored basic dye, a color developer such as phenolic compound for causing the dye to produce a color when heated, a chromogenic sensitivity adjusting agent, a binder, etc. The heat-sensitive recording papers obtained with use of the composition are comparable to those incorporating the conventional calcium carbonate in the effect to remove residue and are superior to the latter in color density, anti-fogging property, resistance to light, etc.

The components of the coating composition for heat-sensitive recording paper other than the above calcium carbonate pigment, i.e. the basic dye, color developer, chromogenic sensitivity adjusting agent, binder, and the like can be a wide variety of those conventionally used for heat-sensitive paper. Typical examples of these components are as follows.

### (a) Colorless to pale-colored basic dyes

Triarylmethane dyes such as 3,3-bis(p-dimethylaminophenyl)-6-dimethylaminophthalide, fluoran dyes such as 3-diethylamino-6-methyl-7-anilinofluoran, spiropyran dyes such as 3-methyl-spiro-dinaphthopyran, diphenylmethane dyes such as N-halophenyl-leucoauramine, thiazine dyes such as benzoylleucomethyleneblue, etc.

### (b) Color developers

Phenolic compounds such as 4-tert-butylphenol, 4-hydroxydiphenoxide, 4,4′-isopropylidenediphenol (bisphenol A), 2,2′-methylenebis(4-chlorophenol) and novolak-type phenolic resins, aromatic carboxylic acids or derivatives thereof such as benzoic acid, p-tert-butyl-benzoic acid, p-hydroxybenzoic acid, methyl p-hydroxybenzoate, isopropyl p-hydroxybenzoate, benzyl p-hydroxybenzoate, lauryl gallate, stearyl gallate, salicylanilide, 5-chlorosalicylanilide, 5-tert-butylsalicylic acid, hydroxynaphthoic acid and zinc or like metal salts of these acids or derivatives thereof.

### (c) Chromogenic sensitivity adjusting agents

Higher fatty acid amides such as palmitic acid amide, stearic acid amide, oleic acid amide, hydroxystearic acid amide, methylolated fatty acid amide, ethylenebis fatty acid amide and methylenebis fatty acid amide.

### (d) Binders

Water-soluble high-molecular-weight compounds such as polyvinyl alcohol, methyl cellulose, carboxymethyl cellulose, hydroxyethyl cellulose, hydroxpropyl cellulose, starch, casein, gelatin and gum arabic.

When required, various auxiliary agents for use in known coating compositions for heat-sensitive paper can be further incorporated into the composition of the invention. Examples of such additives are release agents, defoaming agents, ultravio1et absorbers, fluorescent dyes, coloring dyes, preservatives, etc. When required, another pigment can be added in an amount of up to 20% by weight, based on the total amount of the composition. Examples of useful other pigments are aluminum hydroxide, silica, calcined kaolin, kaolin, talc, urea resin, etc.

The components of the coating composition according to the invention and the proportions (solid contents) thereof can be changed according to the contemplated purpose. Usually, the composition comprises the following proportions (solid contents) of components based on the total solids.

| | |
|---|---|
| Basic dye | 3 to 10 wt.% (preferably 5 to 10 wt.%) |
| Color developer | 15 to 50 wt.% (preferably 20 to 40 wt.%) |
| Chromogenic sensitivity adjusting agent | 6 to 30 wt.% (preferably 10 to 30 wt.%) |
| Binder | 16 to 22 wt.% (preferably 16 to 20 wt.%) |
| Calcium carbonate pigment of the invention | 5 to 60 wt.% (preferably 10 to 55 wt.%) |

The coating composition of the invention can be prepared in a known manner, for example, by the following method. First, the basic dye, color developer and chromogenic sensitivity adjusting agent are each separately milled in an aqueous solution of binder. When a ball mill, for example, is used for this purpose, each component is added to the binder solution usually to a solids concentration of 15 to 30 wt. %, and the mill is operated for 2 days to obtain fine particles of 1 to 5 »m in size. The calcium carbonate pigment of the invention, when required together with other pigments, is dispersed in an aqueous solution of binder in the usual manner using a dispersant to prepare a pigment dispersion containing 20 to 30 wt. % of solids. Subsequently, the pigment dispersion and the aqueous suspensions of finely divided components are mixed together in the conventional manner, giving a coating composition for forming a heat-sensitive recording layer of heat-sensitive paper according to the invention. The composition is in the form of a dispersion containing 15 to 30 wt. % of solids.

The composition is applied to a substrate and dried in the usual manner, and the coated substrate is calendered when required to give heat-sensitive paper. The coating composition of the invention is applied usually in an amount of 3 to 15 g/m², preferably 5 to 10 g/m², calculated as dry weight, although the amount is variable, for example, with the properties of the heat-sensitive paper to be obtained.

Thus, the present invention provides a heat-sensitive recording paper which is characterized in that it comprises a substrate and a heat-sensitive recording layer formed thereon by applying the above coating composition and drying the resulting coating. Examples of useful substrates are various papers, synthetic resin sheets or films and the like which are conventionally used in the art.

### (2) Coating composition for forming an intermediate layer between heat-sensitive recording layer of heat-sensitive recording paper and substrate thereof

Our research has revealed that when the composition containing 5 to 40 parts by weight of a binder per 100 parts by weight of the calcium carbonate pigment of the invention is applied to a substrate to form an intermediate layer and a heat-sensitive recording layer is formed over the intermediate layer, the resulting paper is higher in color density, anti-fogging property, resistance to light, and the like than when the conventional calcium carbonate is used.

The binder to be used for the coating composition for forming the intermediate layer can be any of the binders already mentioned in item (1) for the heat-sensitive recording layer. Also useful are latices of styrene-butadiene copolymer, polyvinyl acetate, polyurethane, polyacrylic acid, polyacrylate, vinyl chloride-vinyl acetate copolymer, polybutyl methacrylate, ethylene-vinyl acetate copolymer, styrene-butadiene-acrylic copolymer and the like. When required, the coating composition may have further incorporated therein other pigments (such as calcined kaolin, silica, etc.), dispersants, surfactants, defoaming agents, coloring dyes, preservatives, etc.

While the proportions of components (calculated as solids) of the coating composition for forming the intermediate layer are variable over a wide range, a binder is used preferably in an amount of, calculated as solids, 5 to 40 parts by weight, preferably 10 to 35 parts by weight, per 100 parts by weight of the calcium carbonate pigment of the invention. The amount of another pigment to be added when required is up to 40 parts by weight, preferably 10 to 40 parts by weight, per 100 parts by weight of the combined amount of the calcium carbonate pigment of the invention and the binder calculated as solids.

The coating composition for the intermediate layer can be prepared by uniformly dispersing the calcium carbonate pigment of the invention and another pigment when so required in an aqueous solution of binder in the usual manner using a dispersant or the like to obtain a pigment dispersion containing 25 to 35 wt. % of solids. The composition can be applied to a substrate by various methods, for example, by a coater such as steel blade, air knife, roll, flexographic press, Mayer bar or the like. The amount of the composition to be applied, although widely variable, is generally 1 to 15 g/m², preferably 3 to 10 g/m², calculated as dry weight. The coating, when dried, is preferably calendered.

A heat-sensitive recording layer is formed by applying the coating composition for forming a heat-sensitive recording layer as stated above in item (1) in the conventional manner to the intermediate layer thus formed, and drying the coating layer, whereby a heat-sensitive recording paper is obtained which is excellent in effect to remove residue, anti-fogging property, color density, resistance to light and other properties.

Accordingly, the present invention further provides a heat-sensitive recording paper comprising a substrate, the above intermediate layer formed thereon and the heat-sensitive recording layer formed over the intermediate layer from the coating composition for a heat-sensitive recording layer which composition contains the calcium carbonate pigment of the invention as described above in item (1). Examples of useful substrates are paper, synthetic resin film and the like which are conventionally used in the art. The heat-sensitive recording layer can be any of those heretofore known other than those described above in item (1), such as one containing a colorless to pale-colored basic dye, color developer, chromogenic sensitivity adjusting agent, binder and the like as exemplified in item (1), and various other layers.

The reason still remains to be clarified why the above calcium carbonate pigment of the invention used for the coating layer of heat-sensitive recording paper produces the above excellent effects. However, the reason could presumably be explained as follows. Calcium carbonate has some characteristics of solid acid as its surface properties, and the surface acidity of solid thereof is considered to be associated with the anti-fogging property of heat-sensitive recording paper. While the surface of particulate calcium carbonate is relatively low in surface acidity of solid, calcium carbonates of greater BET specific surface area tend to have a higher surface acidity of solid. It is assumed accordingly that in a heat-sensitive recording layer, the calcium carbonate pigment of greater BET specific surface area has a larger surface area in contact with a basic dye acting as a chromogenic material, resulting in reduction of anti-fogging property. Calcium carbonate pigments for heat-sensitive paper are also required to have a high oil absorption which is another important property of such pigment. Presumably, by surface-treating the calcium carbonate of 17 to 55 m²/g in BET specific surface area according to the specific surface-treating method of the invention which induces substantially no reduction in the BET specific surface area or the oil absorption, the calcium carbonate pigment of the invention is endowed with a surface acidity of solid in the specific range, and thereby a heat-sensitive recording paper improved in anti-fogging property, color density and effect to remove residue is obtained. The calcium carbonate of the invention used also provides a heat-sensitive recording paper with higher resistance to light. However, the effect is unpredictable from the relation with the surface acidity of solid, and the reason for this improvement remains unclear.

Furthermore, the calcium carbonate of the invention used for heat-sensitive paper can enhance the whiteness and non-transparency of the paper.

The calcium carbonate pigments of the invention also have the following advantages.
1) When used as a filler for paper, the calcium carbonate of the invention can increase the retention of filler and enhance the whiteness and non-transparency of paper.
2) When incorporated into a coating composition for coat paper, the pigment of the invention gives a coating layer having a porous surface which can effectively absorb the applied printing ink, thereby accelerating the drying.

### Examples

The present invention will be described below in more detail with reference to the following examples. In the following examples, "parts" and "percentages" are all by weight unless otherwise specified.

### Example 1

A 100 kg quantity of an aqueous suspension of calcium carbonate having a BET specific surface area of 20 m²/g, adjusted to a concentration of 20 wt.% and a temperature of 20°C, was placed into a reactor equipped with an impeller disperser. Thereafter, 1.4 kg of an aqueous solution of sodium aluminate adjusted to a concentration of 10 wt.% was added to the aqueous suspension with stirring at 500 r.p.m., and the resulting mixture was further agitated for 15 minutes. After completion of the agitation, the aqueous suspension of calcium carbonate was dewatered by a filter press. The solid product obtained was dried, pulverized and classified, giving 20 kg of a calcium carbonate pigment for heat-sensitive recording paper of the present invention.

### Examples 2 to 7

Calcium carbonate pigments for heat-sensitive recording paper of the invention were prepared in the same manner as in Example 1 with the exception of using the conditions listed in Table 2. Table 2 also shows the conditions employed in Example 1.

In Table 2, the calcium carbonates used as starting materials in Examples 1 and 2 were prepared by a process disclosed in Japanese Examined Patent Publication No. 31530/1982, and those used in Examples 3 to 7 were produced by a process set forth in Japanese Unexamined Patent Publication No. 230424/1989.

### Comparative Examples 1 to 5

Comparative calcium carbonate pigments were prepared in the same manner as in Example 1 with the exception of employing the conditions as described below in Table 3. The calcium carbonates used as starting materials in Comparative Examples 1 and 2 were produced by a process disclosed in Japanese Examined Patent Publication No. 31530/1982, and those used in Comparative Examples 3 to 5 were obtained by a process described in Japanese Unexamined Patent Publication No. 230424/1989.

In Comparative Examples 2, 3 and 5, no surface-treating agent was used.

Table 4 below shows the physical properties of the calcium carbonate pigments obtained in Examples 1 to 7 and Comparative Examples 1 to 5.

From the results with respect to Examples 2 and 3 and Comparative Examples 2 and 3 as shown in Table 4, it is revealed that the calcium carbonate pigments of the invention are somewhat increased or decreased in BET specific surface area and oil absorption as compared with calcium carbonate used as the starting material. However, substantially no problem is caused even in the case where the calcium carbonate pigment of the invention is decreased in BET specific surface area or oil absorption. This indicates that the surface acidity of solid of the calcium carbonate pigment of the invention is suppressed to a specific range.

### Example I

Coating compositions for forming the heat-sensitive recording layer of heat-sensitive recording paper were prepared by the following procedure using the calcium carbonate pigments of the invention (those obtained in Examples 1, 3 and 7). The compositions were used for preparing heat-sensitive recording papers.

First, a colorless dye, phenolic compound and fatty acid amide were each separately milled into fine particles according to the following formulations A, B and C. For this purpose, ball mills were operated for 2 days.

| Formulation A | |
|---|---|
| 3-Diethylamino-6-methyl-7-anilinofluoran (product of Yamamoto Kagaku Gosei Co., Ltd., trademark "ONE DYE BLACK") | 100 parts |
| 5% Aqueous solution of polyvinyl alcohol | 500 parts |

| Formulation B | |
|---|---|
| Bisphenol A | 100 parts |
| 5% Aqueous solution of polyvinyl alcohol | 500 parts |

| Formulation C | |
|---|---|
| Fatty acid amide (trademark "ARMID HT-P", product of Lion ARMER Co., Ltd., m.p. 98°C, mixture of 22% palmitic acid amide, 75% stearic acid amide and 3% of oleic acid amide) | 100 parts |
| 5% Aqueous solution of polyvinyl alcohol | 500 parts |

According to the following formulation D, the calcium carbonate pigment of the invention was made into a pigment dispersion containing 25% of solids using an impeller-type agitator.

| Formulation D | |
|---|---|
| Calcium carbonate pigment | 100 parts |
| 5% Aqueous solution of polycarboxylic acid dispersant | 20 parts |
| 5% Aqueous solution of polyvinyl alcohol | 300 parts |
| Water | 40 parts |

The dispersions A to D prepared according to the formulations A to D were mixed together in the ratio by weight of A:B:C:D = 1:5:3:5 to prepare coating compositions of the invention for forming a heat-sensitive recording layer.

Using a coating rod, the coating composition thus prepared was applied to one surface of wood-free paper, weighing 50 g/m², in the usual manner in an amount of 6 g/m² on dry basis. After drying the coating at room temperature, the coated paper was calendered to obtain heat-sensitive paper.

Table 5 showing the characteristics of the paper thus obtained indicates that the paper retains substantially the same degree of whiteness before and after the heating of the paper and is excellent in anti-fogging property. Further, the paper is outstanding in resistance to light and has high effect to remove residue.

### Comparative Example I

Comparative coating compositions for forming a heat-sensitive recording layer were prepared in the same manner as in Example I except that the comparative calcium carbonate pigments obtained in Comparative Examples 1 to 5 were used. The compositions were used for preparing heat-sensitive recording paper. Table 5 shows the characteristics of the paper obtained. Table 5 also shows the results obtained using known calcium carbonate (i) (which is disclosed in Japanese Unexamined Patent Publication No. 230424/1989). The physical properties of the known calcium carbonate (i) used are as follows. (The same applies in the following description.)

| | |
|---|---|
| BET specific surface area | 38 m²/g |
| Surface acidity of solid | 44 »mol/g |
| Oil absorption | 140 ml/100 g |
| Bulk | 10 ml/g |
| Sedimentation volume | 75 ml/60 min |
| Hiding power | 35 cm²/g |
| True specific gravity | 2.60 |

### Example II

Calcium carbonate pigments of the invention (those obtained in Examples 1, 3 and 7) were used for forming the intermediate layer of heat-sensitive paper. More specifically, the calcium carbonate pigment was uniformly dispersed according to the following formulation to obtain a coating composition for forming the intermediate layer.

| | |
|---|---|
| Calcium carbonate pigment | 100 parts |
| 5% Aqueous solution of polycarboxylic acid dispersant | 20 parts |
| 5% Aqueous solution of polyvinyl alcohol | 300 parts |
| Styrene-butadiene latex (brand name "SN-307", product of Sumitomo Naugatuck Co., Ltd., solids content 48%) | 20 parts |
| Water | 40 parts |

Using a coating rod, the coating composition was applied to one surface of wood-free paper, weighing 50 g/m², in the usual manner in an amount of 7 g/m² on dry basis. After drying the coating, the coated paper was falendered to obtain pigment-coated paper.

Dispersions A, B, C and D prepared according to the formulations A to D in Example I were mixed together in the ratio by weight of A:B:C:D = 1:5:3:1 to obtain a coating composition, which was then applied to the pigment-coated paper in an amount of 6 g/m² on dry basis using a coating rod. After drying the coating at room temperature, the resulting paper was calendered to obtain heat-sensitive recording paper having an intermediate layer. Table 5 showing the characteristics of the heat-sensitive recording paper thus prepared indicates that the paper retained substantially the same whiteness before and after the heating of the paper, and was outstanding in anti-fogging property and resistance to light. Further, the paper had sufficiently high effect to remove residue.

### Comparative Example II

Comparative coating compositions for forming an intermediate layer were prepared in the same manner as in Example II except that the comparative calcium carbonates obtained in Comparative Examples 1 to 5 were used. Comparative heat-sensitive paper having an intermediate layer was obtained in the same manner as in Example II using each of the comparative coating compositions. The characteristics of the heat-sensitive recording paper thus obtained were shown in Table 5, which also shows the result achieved using known calcium carbonate (i) similarly.

As clear from the results shown in Table 5, the calcium carbonate pigment of the present invention is excellent not only in anti-fogging property but in resistance to light in comparison with known calcium carbonate pigments.

## Claims

1. A calcium carbonate pigment for heat-sensitive recording paper, the pigment having a BET specific surface area of 17 to 55 m²/g, an oil absorption of 90 to 220 ml/100 g as determined by the Ogura method and a surface acidity of solid represented by the equation (Z):
$\text{y=0.13 x + 31 (Z)}$
wherein x is a BET specific surface area (m²/g) and y is a surface acidity of solid (»mol/g).

2. A calcium carbonate pigment according to claim 1 which has a BET specific surface area of 19 to 55 m²/g.

3. A process for preparing the calcium carbonate pigment of claim 1 for heat-sensitive recording paper, the process comprising the steps of (i) adding a calcium carbonate surface-treating agent to an aqueous suspension of a calcium carbonate having a BET specific surface area of 17 to 55 m²/g, the surface-treating agent being at least one member selected from the group consisting of hydroxide of alkaline earth metal, hydroxide of alkali metal, carbonate of alkali metal, bicarbonate of alkali metal, sodium aluminate, aluminum acetate and acetic acid salt of C₄₋₁₄ aliphatic amine, and (ii) stirring the mixture.

4. A process according to claim 3 wherein the calcium carbonate has a BET specific surface area of 19 to 55 m²/g.

5. A process according to claim 3 wherein the surface-treating agent is used in an amount of 0.1 to 5 parts by weight per 100 parts by weight of the calcium carbonate.

6. A process according to claim 3 wherein the surface-treating agent is used in an amount of 0.2 to 4 parts by weight per 100 parts by weight of the calcium carbonate.

7. A coating composition for forming a heat-sensitive recording layer of heat-sensitive recording paper characterized in that the composition comprises 5 to 60% by weight of the calcium carbonate pigment of claim 1 based on the total solids.

8. A coating composition according to claim 7 which comprises, calculated as solids, 3 to 10 wt.% of a basic dye, 15 to 50 wt.% of a color developer, 6 to 30 wt.% of a chromogenic sensitivity adjusting agent, 16 to 22 wt.% of a binder, and 5 to 60 wt.% of the calcium carbonate pigment of claim 1, based on the total solids.

9. A coating composition according to claim 7 which comprises, calculated as solids, 5 to 10 wt.% of a basic dye, 20 to 40 wt.% of a color developer, 10 to 30 wt.% of a chromogenic sensitivity adjusting agent, 16 to 20 wt.% of a binder, and 10 to 55 wt.% of the calcium carbonate pigment of claim 1, based on the total solids.

10. A coating composition for forming an intermediate layer between a heat-sensitive recording layer of heat-sensitive recording paper and the substrate thereof, characterized in that the composition contains a binder in an amount, calculated as solids, of 5 to 40 parts by weight per 100 parts by weight of the calcium carbonate pigment of claim 1.

11. A heat-sensitive recording paper which comprises a substrate and a heat-sensitive recording layer formed thereon and containing the calcium carbonate pigment of claim 1, a chromogenic sensitivity adjusting agent, a colorless to pale-colored basic dye, a color developer for causing the dye to produce a color when heated and a binder.

12. A heat-sensitive recording paper according to claim 11 characterized in that it is obtained by applying the coating composition of claim 8 to the substrate and drying the coating layer.

13. A heat-sensitive recording paper according to claim 11 characterized in that it is obtained by applying the coating composition of claim 9 to the substrate and drying the coating layer.

14. A heat-sensitive recording paper which comprises (i) a substrate, (ii) an intermediate layer formed thereon and containing the calcium carbonate pigment of claim 1 and (iii) a heat-sensitive recording layer formed on the intermediate layer and containing the calcium carbonate pigment of claim 1, a chromogenic sensitivity adjusting agent, a colorless to pale-colored basic dye, a color developer for causing the dye to produce a color when heated and a binder.

15. A heat-sensitive recording paper according to claim 14 which comprises (a) a substrate, (b) an intermediate layer formed by applying to the substrate the coating composition of claim 10 for forming an intermediate layer and drying the coating layer and (c) a heat-sensitive recording layer formed by applying the coating composition of claim 8 for forming a heat-sensitive recording layer to the intermediate layer and drying the coating layer.

16. A heat-sensitive recording paper according to claim 14 which comprises (a) a substrate, (b) an intermediate layer formed by applying to the substrate the coating composition of claim 10 for forming an intermediate layer and drying the coating layer and (c) a heat-sensitive recording layer formed by applying the coating composition of claim 9 for forming a heat-sensitive recording layer to the intermediate layer and drying the coating layer.

## Patentansprüche

1. Calciumcarbonatpigment für wärmeempfindliches Aufzeichnungspapier, wobei das Pigment eine spezifische Oberfläche gemäß BET von 17 bis 55 m²/g, eine Ölabsorption von 90 bis 220 ml/100 g, ermittelt nach dem Ogura-Verfahren, und eine Oberflächenacidität des Festkörpers, wiedergegeben durch die Gleichung (Z):
$\text{y = 0.13 x + 31 (Z)}$
besitzt, in der x eine spezifische Oberfläche gemäß BET (m²/g) und y eine Oberflächenacidität des Feststoffs (»mol/g) ist.

2. Calciumcarbonatpigment gemäß Anspruch 1, das eine spezifische Oberfläche gemäß BET von 19 bis 55 m²/g besitzt.

3. Verfahren zur Herstellung des Calciumcarbonatpigments gemäß Anspruch 1 für wärmeempfindliches Aufzeichnungspapier, welches die Schritte umfaßt:
(i) Zugabe eines Calciumcarbonat-Oberflächenbehandlungsmittels zu einer wäßrigen Suspension eines Calciumcarbonats mit einer spezifischen Oberfläche gemäß BET von 17 bis 55 m²/g, wobei das Oberflächenbehandlungsmittel mindestens ein Mitglied, ausgewählt aus der Gruppe, bestehend aus einem Hydroxid eines Erdalkalimetalls, einem Hydroxid eines Alkalimetalls, einem Carbonat eines Alkalimetalls, einem Bicarbonat eines Alkalimetalls, Natriumaluminat, Aluminiumacetat und einem Essigsäuresalz eines C₄₋₁₄- aliphatischen Amins, ist und
(ii) Rühren der Mischung.

4. Verfahren gemäß Anspruch 3, worin das Calciumcarbonat eine spezifische Oberfläche gemäß BET von 19 bis 55 m²/g besitzt.

5. Verfahren gemäß Anspruch 3, worin das Oberflächenbehandlungsmittel in einer Menge von 0.1 bis 5 Gew.-Teilen, pro 100 Gew.-Teile Calciumcarbonat, verwendet wird.

6. Verfahren gemäß Anspruch 3, worin das Oberflächenbehandlungsmittel in einer Menge von 0.2 bis 4 Gew.-Teilen, pro 100 Gew. -Teile Calciumcarbonat, verwendet wird.

7. Beschichtungszusammensetzung zur Herstellung einer wärmeempfindlichen Aufzeichnungsschicht eines wärmeempfindlichen Aufzeichnungspapiers, dadurch gekennzeichnet, daß die Zusammensetzung 5 bis 60 Gew.-% des Calciumcarbonatpigments gemäß Anspruch 1 enthält, bezogen auf die gesamten Feststoffe.

8. Beschichtungezusammensetzung gemäß Anspruch 7, welche, berechnet als Feststoffe, umfaßt:
3 bis 10 Gew.-% eines Basisfarbstoffs, 15 bis 50 Gew.-% eines Farbentwicklers, 6 bis 30 Gew.-% eines chromogenen Empfindlichkeitseinstellungsmittels, 16 bis 22 Gew.-% eines Bindemittels und 5 bis 60 Gew.-% des Calciumcarbonatpigments gemäß Anspruch 1, bezogen auf die gesamten Feststoffe.

9. Beschichtungezusammensetzung gemäß Anspruch 7, welche, berechnet als Feststoffe, umfaßt:
5 bis 10 Gew.-% eines Basisfarbstoffs, 20 bis 40 Gew.-% eines Farbentwicklers, 10 bis 30 Gew.-% eines chromogenen Empfindlichkeitseinstellungsmittels, 16 bis 20 Gew.-% eines Bindemittels und 10 bis 55 Gew.-% des Calciumcarbonatpigments gemäß Anspruch 1, bezogen auf die gesamten Feststoffe.

10. Beschichtungszusammensetzung zur Herstellung einer Zwischenschicht zwischen einer wärmeempfindlichen Aufzeichnungsschicht eines wärmeempfindlichen Aufzeichnungspapiers und dessen Träger, dadurch gekennzeichnet, daß die Zusammensetzung ein Bindemittel in einer Menge von 5 bis 40 Gew.-Teilen, pro 100 Gew.-Teile des Calciumcarbonatpigments gemäß Anspruch 1, berechnet als Feststoffe, enthält.

11. Wärmeempfindliches Aufzeichnungspapier, welches einen Träger und eine auf diesem gebildete wärmeempfindliche Aufzeichnungsschicht umfaßt und welche das Calciumcarbonatpigment gemäß Anspruch 1, ein chromogenes Empfindlichkeitseinstellungsmittel, einen farblosen bis schwach gefärbten Basisfarbstoff, einen Farbentwickler, der den Farbstoff veranlaßt, beim Erwärmen eine Farbe zu erzeugen, und ein Bindemittel enthält.

12. Wärmeempfindliches Aufzeichnungspapier gemäß Anspruch 11, dadurch gekennzeichnet, daß es erhalten wird durch Aufbringen der Beschichtungszusammensetzung gemäß Anspruch 8 auf den Träger und Trocknen der Überzugsschicht.

13. Wärmeempfindliches Aufzeichnungspapier gemäß Anspruch 11, dadurch gekennzeichnet, daß es erhalten wird durch Aufbringen der Beschichtungszusammensetzung gemäß Anspruch 9 auf den Träger und Trocknen der Überzugsschicht.

14. Wärmeempfindliches Aufzeichnungspapier, welches umfaßt:
(i) einen Träger, (ii) eine auf diesem gebildete Zwischenschicht, die das Calciumcarbonatpigment gemäß Anspruch 1 enthält, und (iii) eine auf der Zwischenschicht gebildete wärmeempfindliche Aufzeichnungsschicht, welche das Calciumcarbonatpigment gemäß Anspruch 1, ein chromogenes Empfindlichkeitseinstellungsmittel, einen farblosen bis schwach gefärbten Basisfarbstoff, einen Farbentwickler, der den Farbstoff veranlaßt, beim Erwärmen eine Farbe zu erzeugen, und ein Bindemittel enthält.

15. Wärmeempfindliches Aufzeichnungspapier gemäß Anspruch 14, welches umfaßt:
(a) einen Träger, (b) eine Zwischenschicht, gebildet durch Aufbringen der Beschichtungszusammensetzung gemäß Anspruch 10 auf den Träger, um eine Zwischenschicht zu bilden, und Trocknen der Überzugsschicht, und (c) eine wärmeempfindliche Aufzeichnungsschicht, gebildet durch Aufbringen der Beschichtungszusammensetzung gemäß Anspruch 8, um eine wärmeempfindliche Aufzeichnungsschicht auf der Zwischenschicht zu bilden, und Trocknen der Überzugsschicht.

16. Wärmeempfindliches Aufzeichnungspapier gemäß Anspruch 14, welches umfaßt:
(a) einen Träger, (b) eine Zwischenschicht, gebildet durch Aufbringen der Beschichtungszusammensetzung gemäß Anspruch 10 auf den Träger, um eine Zwischenschicht zu bilden, und Trocknen der Überzugsschicht, und (c) eine wärmeempfindliche Aufzeichnungsschicht, gebildet durch Aufbringen der Beschichtungszusammensetzung gemäß Anspruch 9, um eine wärmeempfindliche Aufzeichnungsschicht auf der Zwischenschicht zu bilden, und Trocknen der Überzugsschicht.

## Revendications

1. Pigment à base de carbonate de calcium pour papier d'enregistrement thermosensible, ledit pigment ayant une surface spécifique BET de 17 à 55 m²/g, une valeur d'absorption d'huile de 90 à 220 ml/100 g, telle que déterminée au moyen du procédé de Ogura, et une acidité superficielle de solide représentée par l'équation (Z) :
$\text{y = 0,13 x + 31 (Z)}$
où x est une valeur de surface spécifique BET (m²/g) et y est une valeur d'acidité superficielle de solide (»mol/g).

2. Pigment à base de carbonate de calcium selon la revendication 1, ayant une surface spécifique BET de 19 à 55 m²/g.

3. Procédé de préparation du pigment à base de carbonate de calcium selon la revendication 1 pour papier d'enregistrement thermosensible, comprenant les étapes consistant à (i) ajouter un agent de traitement superficiel du carbonate de calcium à une suspension aqueuse d'un carbonate de calcium ayant une surface spécifique BET de 17 à 55 m²/g, l'agent de traitement superficiel étant au moins un élément choisi dans l'ensemble constitué par les hydroxydes de métaux alcalino-terreux, les hydroxydes de métaux alcalins, les carbonates de métaux alcalins, les bicarbonates de métaux alcalins, l'aluminate de sodium, l'acétate d'aluminium et un sel d'acide acétique d'une amine aliphatique en C₄₋₁₄, et (ii) agiter le mélange.

4. Procédé selon la revendication 3, dans lequel le carbonate de calcium a une surface spécifique BET de 19 à 55 m²/g.

5. Procédé selon la revendication 3, dans lequel on utilise l'agent de traitement superficiel en une quantité de 0,1 à 5 parties en poids pour 100 parties en poids de carbonate de calcium.

6. Procédé selon la revendication 3, dans lequel on utilise l'agent de traitement superficiel en une quantité de 0,2 à 4 parties en poids pour 100 parties en poids de carbonate de calcium.

7. Composition de revêtement pour former une couche d'enregistrement thermosensible à base de papier d'enregistrement thermosensible, caractérisée en ce qu'elle contient de 5 à 60 % en poids du pigment à base de carbonate de calcium selon la revendication 1, par rapport à la quantité totale des solides.

8. Composition de revêtement selon la revendication 7, comprenant, calculés à l'état solide, 3 à 10 % en poids d'un colorant basique, 15 à 50 % en poids d'un révélateur de couleur, 6 à 30 % en poids d un agent d'ajustement de la sensibilité chromogène, 16 à 22 % en poids d'un liant et 5 à 60 % en poids du pigment à base de carbonate de calcium selon la revendication 1, par rapport à la quantité totale des solides.

9. Composition de revêtement selon la revendication 7, comprenant, calculés à l'état solide, 5 à 10 % en poids d'un colorant basique, 20 à 40 % en poids d'un révélateur de couleur, 10 à 30 % en poids d un agent d'ajustement de la sensibilité chromogène, 16 à 20 % en poids d'un liant et 10 à 55 % en poids du pigment à base de carbonate de calcium selon la revendication 1, par rapport à la quantité totale des solides.

10. Composition de revêtement pour former une couche intermédiaire entre une couche d'enregistrement thermosensible formée de papier d'enregistrement thermosensible et le substrat de celle-ci, caractérisée en ce qu'elle contient un liant en une quantité de 5 à 40 parties en poids, calculée à l'état solide, pour 100 parties en poids du pigment à base de carbonate de calcium selon la revendication 1.

11. Papier d'enregistrement thermosensible comprenant un substrat et une couche d'enregistrement thermosensible formée sur celui-ci et contenant le pigment à base de carbonate de calcium selon la revendication 1, un agent d'ajustement de la sensibilité chromogène, un colorant basique incolore ou faiblement coloré, un révélateur de couleur pour obliger le colorant à produire une couleur quand il est chauffé, et un liant.

12. Papier d'enregistrement thermosensible selon la revendication 11, caractérisé en ce qu'on l'obtient en appliquant la composition de revêtement de la revendication 8 sur le substrat et en faisant sécher la couche de revêtement.

13. Papier d'enregistrement thermosensible selon la revendication 11, caractérisé en ce qu'on l'obtient en appliquant la composition de revêtement de la revendication 9 sur le substrat et en faisant sécher la couche de revêtement.

14. Papier d'enregistrement thermosensible comprenant (i) un substrat, (ii) une couche intermédiaire formée sur celui-ci et contenant le pigment à base de carbonate de calcium selon la revendication 1, et (iii) une couche d'enregistrement thermosensible formée sur la couche intermédiaire et contenant le pigment à base de carbonate de calcium selon la revendication 1, un agent d'ajustement de la sensibilité chromogène, un colorant basique incolore à faiblement coloré, un révélateur de couleur pour obliger le colorant à produire une couleur quand il est chauffé, et un liant.

15. Papier d'enregistrement thermosensible selon la revendication 14, comprenant (a) un substrat, (b) une couche intermédiaire formée par application sur le substrat de la composition de revêtement de la revendication 10 pour former une couche intermédiaire et séchage de la couche de revêtement, et (c) une couche d'enregistrement thermosensible formée par application de la composition de revêtement de la revendication 8 pour former une couche d'enregistrement thermosensible sur la couche intermédiaire et séchage de la couche de revêtement.

16. Papier d'enregistrement thermosensible selon la revendication 14, comprenant (a) un substrat, (b) une couche intermédiaire formée par application sur le substrat de la composition de revêtement de la revendication 10 pour former une couche intermédiaire et séchage de la couche de revêtement, et (c) une couche d'enregistrement thermosensible formée par application de la composition de revêtement de la revendication 9 pour former une couche d'enregistrement thermosensible sur la couche intermédiaire et séchage de la couche de revêtement.
